

Oct. 17, 1944.

W. B. ROSS ET AL

2,360,585

MOTOR FUEL

Filed Oct. 27, 1941

3 Sheets-Sheet 1



*Fig. 1*

INVENTORS.

By *William B. Ross*  
*Kenneth Boldt*

ATTORNEY.  
*Edward H. Harrington*

Oct. 17, 1944.

W. B. ROSS ET AL

2,360,585

MOTOR FUEL

Filed Oct. 27, 1941

3 Sheets-Sheet 2



*Fig. 2*

INVENTORS.  
William B. Ross  
BY Kenneth Boldt  
ATTORNEY.  
*Edward H. Ladd*

Oct. 17, 1944.

W. B. ROSS ET AL

2,360,585

MOTOR FUEL

Filed Oct. 27, 1941

3 Sheets-Sheet 3



Fig. 3

INVENTORS  
BY *William B. Ross*  
*Kenneth Boldt*  
*Edward H. Lang*, ATTORNEY.

## UNITED STATES PATENT OFFICE

2,360,585

## MOTOR FUEL

William B. Ross, Evanston, and Kenneth Boldt,  
Highland Park, Ill., assignors to The Pure Oil  
Company, Chicago, Ill., a corporation of Ohio

Application October 27, 1941, Serial No. 416,656

8 Claims. (Cl. 44—80)

This invention relates to motor fuels for internal combustion engines and particularly to automotive gasoline fuels having superior performance characteristics. The invention is particularly directed to providing motor fuels having high susceptibility to improvement by the addition of metallo-organic anti-knock agents such as lead tetraethyl and having high anti-knock quality as well as balanced distillation characteristics.

Among the qualities which characterize good gasoline, high anti-knock rating has probably become the most important. Many efforts have been made to improve the anti-knock value of motor fuels, and for this purpose many substances have been incorporated in gasoline. For example, metallo-organic compounds, benzol and various alcohols have been utilized. More recently, olefin polymers such as the polymers of olefins containing from two to five carbon atoms have been widely used in commercial motor fuels with great advantage. These materials can be prepared from the waste gases produced in the cracking of petroleum oil. The anti-knock properties of the olefin polymers may vary greatly depending upon such factors as the method of manufacture and the particular olefin used. However, it is a general practice today to add lead tetraethyl to hydrocarbon base stocks in order to bring the resultant fuel blend to a uniform high anti-knock value.

Studies of the problem of motor knock and of motor fuel compositions have revealed that the tendency of a motor fuel to cause engine knock is a function of the fuel composition as well as of engine conditions. It has been found that in general, anti-knock value of a homologous series of hydrocarbons depends upon the number of carbon atoms in the molecules and the compactness of the molecular structure, the anti-knock value increasing with numerical decrease and centralization of carbon atoms. The effect of tetraethyl lead on the anti-knock value of motor fuels has also been studied and a characterizing factor called "lead susceptibility" has been introduced. By this factor, fuels may be evaluated in terms of the improvement in anti-knock value effected by a given addition of tetraethyl lead. It has been established that some gasolines show more improvement in anti-knock rating for a given addition of tetraethyl lead than do others. This variation in susceptibility has been found to be related to the composition of the fuel. For example, paraffinic and naphthenic hydrocarbons

in general have been found to be much more susceptible to anti-knock improvement by the addition of tetraethyl lead than olefinic and aromatic hydrocarbons, the lead susceptibility being greatest in the paraffins and diminishing in the other hydrocarbons in the order named.

It has been found that the unusual improvement in performance of internal combustion engines effected by motor fuels in accordance with this invention is not fully indicated by the usual anti-knock rating determination, due to deficiencies inherent in the available recognized methods of testing. Many methods and a rather large number of devices have been proposed for the evaluation of motor fuels by knocking tendencies. Probably the best-known testing devices are the Ricardo variable compression engine, the Ethyl Gasoline Series 30 engine, and the Cooperative Fuel Research engine, usually called C. F. R. The C. F. R. engine is undoubtedly in more general use today than any other engine for anti-knock testing purposes. The most widely used method of determining the knocking tendency with the C. F. R. engine is one which has been standardized and recommended by the American Society for Testing Materials. This is known as the A. S. T. M. Motor Method and is designated Method D 357-40. Results of tests by the A. S. T. M. Motor Method using the C. F. R. engine are reported in terms of octane numbers. Octane number of a motor fuel is numerically equivalent to the percent by volume of iso-octane (2, 2, 4 trimethyl pentane) in a mixture of iso-octane and normal heptane, that is equal in knocking tendency to the fuel under test, the better fuels having the higher numerical values. Unless otherwise indicated, all octane numbers in this specification and in the appended claims are A. S. T. M. octane numbers.

From the inception of the method of testing motor fuels by measurement of knocking tendency, there has been and still is a considerable discrepancy between the rating of fuels as determined by the various testing methods. Furthermore, and of probably still greater importance, is the fact that there still prevails a probably greater discrepancy between the ratings of motor fuels as determined by any of the foregoing methods and the rating of motor fuels as determined by actual road performance tests. One prominent factor, if not the most prominent factor, that contributes to the latter discrepancy is the fact that the prevailing testing methods require the operation of the testing engines at

constant speed and under constant load, whereas the knocking tendency of automotive engines in actual operation is greatest during periods of acceleration. Since the unusual characteristics of motor fuels in accordance with this invention are manifest under conditions of engine acceleration, it is apparent that the usual laboratory testing methods are of little value in evaluating such fuel. The only entirely satisfactory method known at the present time is a much more time-consuming and expensive test carried out in stock automotive engines under conditions of actual road performance. This test is called the "Road rating test." The additional time and expense involved is believed to be justified by the fact that the results of such tests are final and conclusive as to the value of a motor fuel in actual service.

The road rating test consists of the evaluation of motor fuels by means of determining the knocking tendency of standard automobile engines when using the particular test fuel under conditions of actual acceleration performance on the road. Since it is generally accepted that knocking is an indication of inefficient operation, those fuels that show the least tendency to knock are the superior fuels. Through the use of proper instruments and replacing the standard automatic distributor with a manually controlled distributor, the speed attained under full throttle acceleration at which the knock dies out for a given spark advance is determined. This test is repeated for a number of different spark advances. By plotting the highest spark advance attainable without evidence of knocking against R. P. M. of engine or car speed in miles per hour, a curve is obtained which when compared with a curve showing the standard spark advance setting of the engine in which the tests are made, indicates whether or not a given fuel may be expected to knock at various speeds in that particular car when operated with a standard spark advance setting. These determinations are generally made in standard motor cars (with the exception of the distributor) under conditions of actual road operation. However, in order to satisfactorily evaluate fuels of unusually high quality, it has been necessary to modify the stock engines by replacing the usual heads with heads having a higher compression ratio.

It is an object of this invention to provide motor fuels having greatly improved performance characteristics.

It is another object of this invention to provide improved motor fuels having high road rating test values at all speeds.

It is still another object of this invention to provide improved motor fuels which exhibit superior high and low speed performance characteristics in internal combustion engines, particularly during periods of acceleration.

A further object is to provide improved motor fuels in which the chemical composition-boiling range characteristics are controlled within a definite fixed relation.

A still further object is to provide improved motor fuels having unusually high susceptibility to improvement in road performance by addition of lead tetraethyl.

These and other objects of the invention will be apparent from the following detailed description considered in connection with the accompanying drawings, all of the figures of which are graphs showing borderline knock-test results obtained with various motor fuels.

It has been established that vastly improved

road performance characteristics at low speed in internal combustion engines can be secured by incorporating in motor fuel used in internal combustion engines, olefin hydrocarbons boiling within in the approximate range of 100° to 140° F. and having an A. S. T. M. Motor Method octane blending value not substantially less than 110.

As a result of extensive tests in actual motor car operation, it has been found that the modern automobile engine performance under conditions of low speed acceleration is closely related to the composition of the low boiling portion of the motor fuel used in the engine, that is, the portion boiling not substantially above 140° F.

15 Likewise, it has been found that the high speed performance of the engine is most closely related to the composition of the higher boiling portion of the motor fuel used in the engine, that is, the portion boiling above about 235° F.

20 The intermediate portion of the fuel boiling between approximately 140° F. and 235° F. may contain any convenient mixture of hydrocarbons so long as the overall octane of this fraction is sufficient to produce the desired overall octane in the finished motor fuel. The proportions of the low boiling, intermediate and high boiling fractions which are used are such as to produce a balanced volatility in the final fuel. An unusually large proportion of either the light fraction or the heavy fraction would lead to uneven carburetion and consequent loss of efficiency in motor performance. A fuel of well balanced volatility capable of producing particularly good all speed performance preferably contains about 8 to 30% by volume of the low boiling fraction, about 20 to 50% by volume of intermediate fraction, and about 35 to 70% by volume of high boiling fraction. It will be appreciated that a fairly wide tolerance in the proportions of these 25 fractions is required in order to prepare motor fuels, the volatility of which is adapted to satisfactory engine operation under both high temperature and low temperature operating conditions.

30 40 45 It has now been found that motor fuels containing predominant amounts of unsaturated hydrocarbons in the low boiling range and not more than minor amounts of unsaturated hydrocarbons particularly unsaturated aliphatic hydrocarbons in the high boiling range, i. e. less than 25% and preferably less than 10% by volume, produce exceptionally good low and high speed performance in internal combustion engines and particularly those engines of high compression ratios such as compression ratios of

50 55 60 about 6.5:1 to 9:1. This is particularly true when the high boiling portion of the fuels contains substantial amounts, for example, about 30% or 50% or more by volume of alkylated benzene hydrocarbons. In the low boiling range those unsaturated hydrocarbons such as monoolefins having a minimum tendency to form undesirable gums are preferred. The maximum boiling points of the constituents in the high boiling fraction should be such that when the constituents are blended with the remaining components of the motor fuel, the end point of the blended fuel will not be substantially in excess of that of ordinary commercial gasoline which

65 70 75 at the present time is in the neighborhood of 400° F. The minimum boiling point of the constituents in the low boiling fraction is largely dependent upon the vapor pressure of the constituents and the characteristics of the remaining fractions of the motor fuel with which the

low boiling materials are blended. Excessive vapor pressure in the finished motor fuel must be avoided since this leads to high storage and transfer losses and to engine operating difficulties commonly known as vapor locking.

In order to show the unusual results in motor performance secured from fuels prepared in accordance with this invention, special fuels were prepared in which the chemical composition-boiling range relationship was controlled within the desired limits and road rating test data on these fuels obtained. In considering these data, it should be borne in mind that not only the road anti-knock qualities of the base gasoline are important, but in addition the response of the fuels to additions of lead tetraethyl are also of great importance since most commercial motor fuels have this anti-knock agent added to them to secure and maintain the desired level of anti-knock value in the finished fuels. It is essential that the leaded fuel as well as the hydrocarbon motor fuel base show the desired road performance characteristics. The data in Table I show the boiling range-chemical composition relationship of the fuels employed in the road rating tests.

Table I

| Fuel No. | Fraction         | Percent by vol. total fuel | Percent by volume of fraction |            |         |           |
|----------|------------------|----------------------------|-------------------------------|------------|---------|-----------|
|          |                  |                            | Parafins                      | Naphthenes | Olefins | Aromatics |
| 2.       | I. B. P.-140° F. | 8                          | 86                            | 14         | 0       | 0         |
|          | 140-235° F.      | 71                         | 72                            | 26         | 0       | 2         |
|          | 235-E. P.        | 21                         | 59                            | 24         | 0       | 17        |
| 3.       | I. B. P.-140° F. | 17                         | 48                            | 0          | 52      | 0         |
|          | 140-235° F.      | 25                         | 25                            | 17         | 45      | 13        |
|          | 235-E. P.        | 59                         | 35                            | 6          | 8       | 51        |
| 4.       | I. B. P.-140° F. | 16                         | 79                            | 0          | 21      | 0         |
|          | 140-235° F.      | 41                         | 14                            | 50         | 4       | 33        |
|          | 235-E. P.        | 43                         | 35                            | 14         | 9       | 42        |
| 5.       | I. B. P.-140° F. | 22                         | 27                            | 0          | 73      | 0         |
|          | 140-235° F.      | 33                         | 20                            | 18         | 59      | 3         |
|          | 235-E. P.        | 45                         | 0                             | 68         | 23      | 8         |
| 8.       | I. B. P.-140° F. | 21                         | 71                            | 0          | 29      | 0         |
|          | 140-235° F.      | 37                         | 41                            | 20         | 39      | 0         |
|          | 235-E. P.        | 42                         | 33                            | 26         | 27      | 14        |
| E-19.    | I. B. P.-140° F. | 8                          | 88                            | 12         | 0       | 0         |
|          | 140-235° F.      | 40                         | 29                            | 30         | 7       | 4         |
|          | 235-E. P.        | 52                         | 27                            | 19         | 11      | 43        |
| E-20.    | I. B. P.-140° F. | 14                         | 38                            | 0          | 62      | 0         |
|          | 140-235° F.      | 34                         | 26                            | 11         | 51      | 12        |
|          | 235-E. P.        | 52                         | 24                            | 12         | 16      | 48        |

Fuel 2 is a blend of standard reference fuels, A-6 (23%) and C-12 (77%), to produce a 70 octane number blended fuel. This fuel was used in the tests as a reference fuel and to show that octane number alone is not indicative of the performance characteristics of a motor fuel. Fuel 3 was prepared by blending 50% by volume of the I. B. P.-275° F. fraction of vapor phase thermal cracked gasoline with 50% by volume of a 200 to 400° F. cut of hydroformed gasoline. This fuel had an A. S. T. M. motor method octane number of 73.5. Fuel 4 was prepared by blending 50% by volume of a mixture of 275° F. end point high pressure cracked gasoline and catalytically dehydrogenated light straight run gasoline with 50% by volume of high boiling fractions of gasoline which had been hydroformed. This fuel had an octane number of 71. Fuel 5 was prepared by blending 50% by volume of I. B. P.-275° F. fraction of vapor phase thermal cracked gasoline with 50% by volume of a 275 to 400° F. cut of naphthenic naphtha obtained from Mirando crude. The octane number of this fuel was 72.3. Fuel 8 was prepared by blending 70% by volume cracked gasoline produced on a combination high pressure cracking unit and 30% by volume of a 325-E. P. cut of

straight run gasoline. This fuel had an octane number of 66.7. Fuel E-19 was prepared by blending 50% by volume of a mixture of low boiling straight run gasoline obtained from Coronado crude oil and 14 pound Reid vapor pressure casing head gasoline with 50% by volume of a mixture containing approximately 90% hydroformed gasoline boiling between 235 and 400° F. and about 10% of a commercial grade of xylene. This fuel had an octane number of 75.3. Fuel E-20 was prepared by blending 50% by volume of the I. B. P. to 235° F. cut of vapor phase thermal cracked gasoline with 50% by volume of the same heavy fraction as was used in fuel E-19. Fuel E-20 had an octane number of 75.6. In the 235-E. P. fraction of all of the fuels, the "Aromatics" indicated in Table I are alkyl benzenes. The analysis of the fuels for the determination of the paraffinic, naphthenic, olefinic and aromatic constituents was carried out in accordance with the method described by Kurtz and Headington, Ind. Eng. Chem., Anal. Ed. 9, 21 (1937).

The curves shown in Figures 1, 2 and 3 forming a part of this specification are curves obtained by the borderline knock test method which is described by Campbell, Greenshield and Holaday in the Journal of the Society of Automotive Engineers, vol. 48, page 193, 1941. These curves clearly show the ability of a fuel to tolerate spark advances without knocking throughout the usual operating speed range. The borderline knock test curves indicate the line which is drawn between satisfactory and unsatisfactory engine operation. When the borderline knock test curve is compared with a curve showing the standard spark advance, the vertical distance between the curves is a measure of the performance quality of the fuel. When the test curve lies above the curve showing the standard spark advance of the particular engine under consideration, satisfactory or non-knocking operation is obtained, whereas when the borderline curve is below the standard spark advance curve, unsatisfactory or knocking performance is obtained. Because of the unusually good performance characteristics of some of the fuels tested, special high compression heads had to be used in order to secure knocking performance. The standard spark advance curves are therefore of very little value and have not been included except in Figure 1, since the standard curves are intended to apply only when using standard engine heads. The engine used in obtaining the tests shown in Figure 1 had a standard head. In all of the curves shown, those having the highest vertical position give the best road performance. In Figure 1, curve 1 shows the standard spark advance setting for the particular car used in the tests. This car was a well-known and widely distributed standard make of motor car, the only deviations from standard equipment being the distributor which permitted manual adjustment of the spark advance. The compression ratio in this engine was 6.5 to 1. Curve 2 shows the results obtained when using fuel 2 which is a 70 octane reference fuel. It will be seen that while the high speed portion of this curve occupies a high vertical position and lies well above curve 1, thus indicating good high speed performance, the left-hand or low speed portion of the curve lies below curve 1, indicating that knocking performance would be obtained at low speeds. Curve 3 shows the results obtained when using fuel 3. This fuel contained a predominant proportion of olefins in the low boiling range, a rela-

tively low proportion of olefins in the high boiling range and a predominant proportion of aromatics in the high boiling range. It will be seen by the vertical distance between curve 2 and curve 3, that fuel 3 has superior performance qualities throughout the entire speed range, the superiority of fuel 3 being most pronounced in the low speed range. Fuel 3 would not cause knocking in this car at any speed and could satisfactorily be used in an engine of unusually high compression ratio.

Curve 4 shows that the high speed performance of fuel 4 is quite satisfactory but that the low speed performance is unsatisfactory in that a knocking operation was obtained when operating the engine at speeds of about 700 to 1100 R. P. M. Although the overall octane of fuel 4 is fairly high, namely 71, unsatisfactory operation in the low speed range was obtained. This can be accounted for by the fact that the low boiling portion of this fuel contains only 21% of olefinic hydrocarbons, the remainder of the fraction being paraffinic hydrocarbons. The high boiling portion of the fuel contains only a small amount of olefins, namely, 9% and contains 42% of aromatics and, therefore, produces a satisfactory high speed performance in spite of the unsatisfactory composition of the low boiling portion of the fuel.

Curve 5 shows that fuel 5 has excellent performance characteristics at both high and low speeds and would not cause knocking in this engine at any speed. This fuel contains 73% by volume of olefins in the low boiling portion and is, therefore, particularly well adapted to produce good operating characteristics in the low speed range. The high boiling portion contains only 23% olefinic hydrocarbons, the remainder being naphthenic and aromatic hydrocarbons. This composition in the high boiling portion of the fuel produced an excellent high speed operation.

The car used to obtain the tests shown in Figure 2 was a standard make of car equipped with a special distributor and a special head. Standard equipment included 14 mm. spark plugs. The compression ratio of the engine was 8 to 1. The tests represented by the curves in Figure 2 were obtained under different climatic conditions and in an entirely different car having a different compression ratio than those shown in Figure 1 and the data in the two figures are, therefore, not directly comparable. Fuels 4, 4b and 4c are all identical as to the hydrocarbon base stock employed, fuel 4 being the clear unleaded fuel, while fuels 4b and 4c are blended fuels containing lead tetraethyl. Similarly, fuels 8, 8b and 8c are identical as to the hydrocarbon base stock employed, fuel 8 being the clear unleaded base stock and fuels 8b and 8c containing lead tetraethyl. The amounts of lead tetraethyl added and the octane numbers of these fuels are shown in Table II.

Table II

| Fuel No. | Ccs. of lead tetra-ethyl per gal. | Octane number<br>motor<br>method |
|----------|-----------------------------------|----------------------------------|
| 4        | 0                                 | 71.0                             |
| 4b       | 0.5                               | 77.2                             |
| 4c       | 1.5                               | 82.0                             |
| 8        | 0                                 | 66.7                             |
| 8b       | 0.5                               | 69.8                             |
| 8c       | 1.5                               | 74.7                             |

It will be noted from the data in Table II that

the lead susceptibility of fuel 4, as shown by the octane number determinations is substantially better than that of fuel 8. This is very unusual in view of the composition of these fuels as indicated in Table I. The data there indicate that fuel 8 is much higher in those components which are generally accepted as having higher lead susceptibility. Fuel 8 is higher in paraffin hydrocarbons and is much lower in aromatic hydrocarbons, the latter being generally regarded as having inferior lead susceptibility characteristics.

The improvement in road performance of fuel 4 effected by the addition of lead tetraethyl, as indicated by the borderline knock test curves shown in Figure 2, is even greater than the improvement in octane number. A comparison of the vertical distance between curves 4 and 4b with the vertical distance between curves 8 and 8b, clearly shows that the road performance of fuel 4 was improved much more by the addition of 0.5 cc. of lead tetraethyl per gallon than was fuel 8. The addition of this amount of lead improved fuel 8 only very slightly, the improvement being entirely confined to the high speed range, whereas the same amount of lead improved fuel 4 over the entire speed range, although the improvement was much greater at speeds of 1500 R. P. M. and higher. A similar but even greater difference may be noted by comparing curves 4 and 4c with 8 and 8c. The improvement effected by the addition of 1.5 cc. of lead tetraethyl per gallon in fuel 4, as indicated by the vertical distance between curves 4 and 4c, is many times greater than the improvement effected by adding the same amount of lead to fuel 8, as shown in curve 8c. Thus, equivalent amounts of lead tetraethyl improved fuel 4 vastly more than the improvement effected by equivalent amounts of lead tetraethyl in fuel 8. This degree of susceptibility to improvement by the addition of lead tetraethyl is of great importance in preparing commercial motor fuels. A further point which is brought out by these curves is the fact that although 1.5 cc. of lead tetraethyl per gallon in fuel 4 produced substantial improvement in both the high speed and low speed ranges, whereas the addition of the same amount of lead tetraethyl to fuel 8 produced scarcely any improvement up to speeds of 1000 R. P. M. This is due to the fact that the low boiling portion of the fuel contained 79% paraffinic hydrocarbons, whereas it has been found that to obtain superior low speed performance, the low boiling portion of the fuel must be predominantly olefinic in character. The high speed performance obtained with fuels 8, 8b and 8c was greatly inferior to that obtained with fuels 4, 4b and 4c, only the high speed portion of fuel 8c being in a superior performance range.

The road rating lead susceptibility of the high speed performance of fuel 4 is all the more remarkable when considered in the light of the composition of the high boiling portion of this fuel. A comparison of the composition of the high boiling portion of this fuel with that of fuel 8, shows that the content of paraffinic hydrocarbons is about the same in both fuels while this fraction of fuel 8 contains higher proportions of naphthenes than does fuel 4 and as previously mentioned, these materials are generally considered to have better lead susceptibility than aromatic hydrocarbons. However, the higher proportion of aromatic hydrocarbons in fuel 4 actually aided in producing a much higher road performance lead susceptibility. This effect is

even more noticeable in those fuels in which the low boiling fraction contains a preponderance of olefinic hydrocarbons.

The unusual road rating lead susceptibility of fuels containing predominant proportions of olefinic hydrocarbons in the low boiling fraction and dominant proportions of aromatics in the high boiling fraction, the high boiling fraction containing not more than small proportions of olefinic hydrocarbons is clearly brought out in Figure 3 which shows a comparison of the data obtained when using fuels E-19 and E-20. The car used to obtain the tests shown in Figure 3 was also a standard model of a widely distributed and well-known brand, although not produced by the same manufacturer as the car employed in obtaining data shown in Figures 1 and 2. The car employed in obtaining the data shown in Figure 3 was equipped with a special head and had a compression ratio of 8.2 to 1. Fuels designated as E-19, E-19b and E-19c are all identical as to the hydrocarbon base stock employed; fuel E-19 being the clear unleaded fuel while fuels E-19b and E-19c are blended fuels containing lead tetraethyl. Similarly, fuels E-20, E-20b and E-20c are identical as to the hydrocarbon base stock employed; fuel E-20 being the clear unleaded base stock and fuels E-20b and E-20c containing lead tetraethyl. The amounts of lead tetraethyl and the octane numbers of these fuels are shown in Table III.

Table III

| Fuel No. | Ccs. of lead tetraethyl per gallon | Octane number motor method |
|----------|------------------------------------|----------------------------|
| E-19     |                                    | 75.3                       |
| E-19b    | 0.5 cc. T. E. L./gal.              | 81.2                       |
| E-19c    | 1.5 cc. T. E. L./gal.              | 86.7                       |
| E-20     |                                    | 75.6                       |
| E-20b    | 0.5 cc. T. E. L./gal.              | 79.9                       |
| E-20c    | 1.5 cc. T. E. L./gal.              | 83.0                       |

It will be noted from the data in Table III that the lead susceptibility of fuels E-19b and E-19c is superior to the lead susceptibility of fuels E-20b and E-20c, respectively. This is presumably due to the high paraffin content of fuels E-19b and E-19c since it is well known that paraffinic hydrocarbons, generally speaking, show a superior lead susceptibility to comparable hydrocarbons of the olefinic, naphthenic or aromatic type. However, a comparison of the road performance tests shown in Figure 3 shows that the performance of fuels E-20, E-20b and E-20c are in general superior to the performance of fuels E-19, E-19b and E-19c, respectively. Note, for example, that the low speed performance of fuel E-20 is considerably better than the low speed performance of fuel E-19, although the overall octane number of these two fuels is substantially the same. The addition of 0.5 cc. of lead tetraethyl to fuel E-20 improved the performance of this fuel over the entire speed range. The improvement in the low speed performance is particularly conspicuous in comparison with the improvement in low speed performance effected by the addition of the same amount of lead tetraethyl to fuel E-19. A comparison of the low speed range of fuels E-20b and E-19b shows that E-20b is far superior to fuel E-19 in this critical low speed range which is the range in which the greatest amount of difficulty with knocking performance in actual operation is ordinarily obtained. A similar but even greater difference pre-

vails in the low speed operation obtained with fuels E-20c and E-19c, the low speed performance of fuel E-20c being vastly superior to the performance obtained with fuel E-19c in the same speed range. The unusual road rating lead susceptibility of fuel E-20 is due to the particular combination of hydrocarbons employed in the low boiling and high boiling portions of this fuel. It is only when fuels contain predominant proportions of olefins in the low boiling range in combination with dominant and preferably preponderating proportions of aromatics in the high boiling portion that such unusual road rating lead susceptibility is obtained. As previously pointed out, the high boiling portion of the fuel must also contain not more than a minor amount such as 10% or 25% of olefinic hydrocarbons.

The particular proportion of unsaturated hydrocarbon components which it is desired to have present in the low boiling fraction of the fuel and the maximum amount of unsaturated aliphatic hydrocarbon components which may be tolerated in the high boiling fraction of the fuel may be varied between rather wide limits as long as the unsaturated hydrocarbons preponderate in the low boiling fraction and the unsaturated aliphatics do not exceed a minor portion in the high boiling fraction. Particularly effective results have been obtained when the low boiling fraction contains a minimum of about 80% olefins and the high boiling fraction preferably contains not over about 25% unsaturated aliphatic hydrocarbons by volume and preferably a maximum of about 10% unsaturated aliphatic hydrocarbons. The high boiling fraction is preferably of relatively high octane number, that is, not less than about 50. Unusually good fuels are those fuels which contain not more than the aforementioned proportions of unsaturated aliphatic hydrocarbons in the high boiling range and in which the high boiling fraction is composed predominantly or substantially of alkylated benzenes. Increased percentages of the components indicated in each case ordinarily produce further improvements. Under present manufacturing conditions it is neither economical nor necessary to have the low boiling fraction consist entirely of olefins or the high boiling fraction entirely free of unsaturated hydrocarbons.

By thus controlling the chemical composition-boiling range characteristics of motor fuels, it is possible to obtain greatly improved engine performance. It is possible to effect these unusual results either by adding hydrocarbon compounds of the desired character and boiling range to motor fuels or by appropriate fractionation and thermal treatment of hydrocarbons and employing the hydrocarbon mixtures thus produced. Small amounts of lead tetraethyl are unusually effective in improving the road performance of the preferred fuels. For a given octane rating, whether it be high or low, motor fuels, the composition of which have been controlled in accordance with this invention produce vastly superior performance in the spark ignition type of internal combustion engines. In general, it is preferred to have a minimum of approximately 65 octane number in the unleaded motor fuel in order to secure most effective results in internal combustion engines now commercially prevalent.

Although the invention has been described in connection with specific details of certain embodiments thereof, it is not intended that such details shall be considered as limiting the scope

of the invention except insofar as indicated in the following claims.

We claim:

1. A motor fuel consisting substantially only of mono-olefinic, paraffinic, naphthenic and aromatic hydrocarbons approximating gasoline in boiling range in which the fraction boiling up to approximately 140° F. comprises 8-30% by volume of the fuel and contains a minimum of 80% of mono-olefins, the fraction boiling above about 235° F. comprises 35-70% of the fuel by volume and contains 50% or more alkyl benzenes, not more than 10% olefins and the balance saturated hydrocarbons, and the overall octane of the fuel is more than 65.

2. A hydrocarbon motor fuel of gasoline boiling range consisting substantially only of mono-olefinic, paraffinic, naphthenic and aromatic hydrocarbons, the portion of said fuel boiling up to about 140° F. comprising from 8 to 30% by volume of said fuel and containing more than 50% of mono-olefinic hydrocarbons, the portion of said fuel boiling from about 140-235° F. comprising from 20-50% by volume of said fuel and the fraction boiling above about 235° F. comprising from 35-70% by volume of said fuel and containing at least 30% of alkylated benzene hydrocarbons, less than 25% of olefinic hydrocarbons and the balance saturated hydrocarbons, said fuel having an over-all A. S. T. M. octane number of not less than 65.

3. A motor fuel in accordance with claim 2 in which the fraction boiling above 235° F. contains less than 10% by volume of olefinic hydrocarbons.

4. A motor fuel consisting of paraffinic, naphthenic, mono-olefinic and aromatic hydrocarbons, approximately 17% by volume of which hydrocarbons constitutes a fraction boiling up to 140° F., the mono-olefinic content of which fraction is approximately 52% by volume, 25% by volume of said fuel constituting a fraction boiling from approximately 140-235° F. and approximately 59% by volume of said fuel constituting a fraction boiling above about 235° F., said last mentioned fraction containing about 51% by volume of aromatic hydrocarbons, about 8% by volume of olefins and the remainder saturated hydrocarbons, said fuel having an A. S. T. M. motor method octane number of 73.5.

5. A hydrocarbon motor fuel of gasoline boiling range substantially free of hydrocarbons other than mono-olefins, paraffins, naphthenes and aromatics, the fraction boiling up to about 140° F. constituting from 8 to 30% by volume of the fuel and containing more than 50% mono-olefins, the fraction boiling between about 140 and 235° F. constituting from 20 to 50% by volume of the fuel and the fraction boiling from about 235° F. to the end point constituting from 35 to 70% by volume of the fuel and containing less than 25% by volume of olefins and a predominant amount of alkyl benzenes, the octane number of the fuel being not less than 65.

15 6. Motor fuel in accordance with claim 5 in which the fraction boiling from about 235° F. to the end point contains less than 10% by volume of olefins.

20 7. A motor fuel consisting substantially only of mono-olefins, naphthenes, paraffins and aromatics within the gasoline boiling range in which the fraction boiling up to about 140° F. constitutes about 22% by volume of the fuel and contains about 73% of mono-olefins and the fraction boiling from about 235° F. to the end point of the fuel constitutes about 45% by volume of the fuel and contains about 23% of mono-olefins, the balance of said fraction consisting of naphthenes and alkyl benzenes, the octane number of the fuel being approximately 72.3.

25 8. A motor fuel consisting substantially only of mono-olefins, paraffins, naphthenes and aromatics within the gasoline boiling range in which the fraction boiling up to about 140° F. constitutes about 14% by volume of the fuel and contains about 62% by volume of olefins, the fraction boiling between about 140 and 235° F. 30 constitutes about 34% by volume of the fuel and the fraction boiling between about 235° F. and the end point constitutes about 52% by volume of the fuel and contains about 48% by volume of alkyl benzenes, about 16% by volume of olefins and the balance saturated hydrocarbons, the 35 octane number of the fuel being about 75.6.

WILLIAM B. ROSS.  
KENNETH BOLDT.